

# United States Patent

Ben et al.

[15] 3,667,207

[45] June 6, 1972

[54] **CRIMPABLE COMPOSITE POLYAMIDE YARN**

[72] Inventors: Victor Ralph Ben, Wilmington, Del.; Peter Steven Kay, Martinsville, Va.

[73] Assignee: E. I. du Pont de Nemours and Company, Wilmington, Del.

[22] Filed: May 1, 1970

[21] Appl. No.: 33,955

[52] U.S. Cl. .... 57/140 BY, 28/72.17, 161/173,  
264/171

[51] Int. Cl. .... D02g 3/02

[58] Field of Search..... 161/173, 175, 177; 260/78 A,  
260/78 L; 57/140 R, 140 BY; 264/DIG. 26;  
28/72.17

[56] References Cited

## UNITED STATES PATENTS

3,554,980 1/1971 Ando et al. .... 264/176 F  
3,322,731 5/1967 Cook et al. .... 260/78 L

3,526,571 9/1970 Ogata..... 264/DIG. 26  
3,418,199 12/1968 Anton..... 161/173  
3,399,108 8/1968 Olson..... 161/173

Primary Examiner—Robert F. Burnett  
Assistant Examiner—Linda C. Koeckert  
Attorney—J. R. McGrath

[57] **ABSTRACT**

A crimpable bicomponent filament in which one component is a polyamide and the other a random copolyamide containing specified percentages of three polymeric units. The different units and their concentrations are 70-82 percent hexamethylene adipamide, 13-25 percent caproamide and 5-17 percent hexamethylene dodecanedioamide. Yarns of one or more such filaments are particularly useful in the manufacture of hosiery because of their high crimpability, high strength and low shrinkage in the fabric.

5 Claims, No Drawings

## CRIMPABLE COMPOSITE POLYAMIDE YARN

## BACKGROUND OF THE INVENTION

This invention relates to composite filaments and particularly to improved composite filaments prepared from synthetic linear polyamides.

Synthetic polyamide filaments and yarns have been predominant in the women's hosiery market for many years. In this market, there is now an increasing demand for the so-called stretch hose. Hose of this type are much smaller than conventional hose but have the ability to stretch much more and thereby provide improved fit as well as reducing the number of sizes of hose required to fit the range of leg sizes normally encountered.

Composite filaments which are particularly suitable for the production of stretch hosiery were disclosed by Olson in U.S. Pat. No. 3,399,108. These filaments have the ability to crimp under restraint and this leads to distortion of the stitches in the hosiery fabric so that the fabric has more ability to stretch than a conventional hosiery fabric. Although these composite filaments have produced good stretch hose, further improvements in crimpability under fabric restraint are desirable, particularly in the production of miniature stretch hose. In this connection, the current wide-spread use of pantyhose also makes improvement in the crimpability of multifilament welt-type yarns very desirable. In addition, improvement in filament strength is desirable in order to enhance the durability of hosiery leg yarns.

## SUMMARY OF THE INVENTION

It is the principal object of this invention to provide a composite polyamide filament having an improved balance of crimp characteristics and strength. Other objects will become apparent from the description and examples to follow.

The above object is accomplished by a crimpable composite filament having a crimp elongation, when subjected to steam at 100° C. under a load of 1.2 milligrams/denier (mgd), greater than 30 percent and consisting of two continuous, adherent, eccentrically arranged, synthetic, polyamide components, one component consisting essentially of a homopolyamide and the other component consisting essentially of a random copolyamide containing at least 70 percent by weight of hexamethylene adipamide units. The copolyamide is characterized by an amide group frequency of 8440-8725 equivalents/10<sup>6</sup> grams and a differential thermal analysis (DTA) melting point of 210°-225° C. Preferably, the homopolyamide is poly(hexamethylene adipamide) i.e., 6-6 nylon, or poly(epsilon-caprolactam), i.e., 6 nylon; and the copolyamide is a copolymer consisting essentially of 70-82 percent by weight of 6-6 nylon polymer units, 13-25 percent by weight of 6 nylon polymer units and 5-17 percent by weight of hexamethylene dodecanedioamide (6-12 nylon) polymer units.

The crimp diameter, i.e., the average diameter of the helices formed when the filament is subjected to steam at 100° C. under a load of 1.2 mgd, is preferably less than 6 mils and most desirably in the range of 3-5 mils.

The copolymer employed should contain at least 70 percent by weight of 6-6 polymer units to provide a high level of strength and durability in hose. The other components of the copolymer should be selected to give a DTA melting point no greater than 225° C. so that the copolymer component of the as-drawn filament will have adequate shrinkage to produce high levels of crimp. The DTA melting point should be at least 210° C. to provide adequate shrinkage tension for crimp formation under restraint and to insure a high tenacity. The amide group frequency should be in the range of 8440-8725 equivalents/10<sup>6</sup> gms. of polymer since lower levels lead to inadequate crimpability and higher levels lead to undesirable moisture sensitivity and loss of fit at high humidity.

The filaments of this invention are prepared by extruding the homopolyamide and copolyamide in either a side-by-side or a sheath-core relationship to form a filament (or two or

more filaments as a yarn), quenching and drawing the filament in the conventional manner, passing the drawn filament through a heating zone under low tension to develop crimp and thereafter stretching the filament to remove crimp. After passing through the heating zone, the crimped filament should be permitted to cool before crimp is removed. The temperature in the heating zone should be at least 140° C. to give the desired crimp characteristics. The temperature required will, of course, depend on the length of the heating zone and the speed of the filament passing through the zone.

The preferred technique for reducing tension in the heating zone and then removing crimp is by passage of the precrimped filament over a series of snubbing pins in its advance away from the draw roll, a suitable heating means such as an air jet being interposed between the draw roll and snubbing pins, as shown, for example, in FIGS. 1 and 4 of the Olson patent. From the snubbing pins, the filament passes around a power-driven roll, rotating at a lower peripheral speed than the draw roll to permit the filament to retract between the rolls. The degree of retraction permissible will depend on the amount of shrinkage, independent of crimping, which occurs between the two rolls. This, in turn, will depend to a considerable extent on the temperature in the heating zone. Generally, a high degree of snubbing is desired to provide very low tension and maximum shrinkage in the heating zone.

In the extrusion of sheath-core filaments, the homopolyamide is preferably extruded as the sheath to facilitate quenching of the filaments. Use of the copolyamide as a sheath results in slower quenching and can lead to filament sticking at high spinning speeds.

The two components are usually present in approximately equal amounts by weight of the filaments; however, the ratio may be varied as required to achieve the desired properties.

With sheath-core filaments, it may be desirable to employ a somewhat larger percentage of the higher shrinkage component in the core.

In producing sheath-core filaments, the core should be highly eccentric in order to develop the required retractive force on crimping. This means that part of the sheath will be very thin, i.e., the minimum thickness of the sheath will range from 5 percent of the filament diameter to 0.1 percent or less.

Either or both of the components may contain any of the various additives commonly employed in the production of fibers, such as delusterants, pigments, dyes, antioxidants, anti-static agents and surface-modifying agents.

In addition to the exemplified yarns, other deniers and other filament counts may be employed. Although hosiery filaments are usually of round cross section, other shapes may be employed and may be particularly useful in certain end uses such as in tricot knit fabrics or certain woven fabrics. For such purposes, cross sections of trilobal shape, shield shape, heart shape, cruciform shape and various multilobal configurations may be employed.

The filaments and yarns of this invention possess an unusually good balance of desirable crimp characteristics, high strength and low shrinkage in the fabric. While certain copolymer compositions outside the limits of this invention may be processed to give almost equivalent crimp characteristics, this is accomplished only at the expense of a loss in strength, particularly after boil-off as in a finished hose. In addition, the filaments of this invention have the desirable characteristic of being essentially straight when removed from the package but tend to develop crimp readily after knitting due to the mechanical working of the filament in the knitting machine. This results in a reduction in area of the greige fabric and, as a consequence, fewer picks develop in the hose during mill handling. Picks are flaws in the stitch construction and may be slight distortions of the stitch which can be corrected by pulling a wale or course or they may be severe distortions which are more difficult to repair.

Surprisingly, the shrinkage of the filaments of this invention is substantially lower than that of prior art bicomponent hosiery filaments. Shrinkages below 4% are readily

achieved. This permits the knitting of a tighter fabric which is less subject to picking and is appreciably more economical in terms of yarn required to provide any given size of hose.

It has also been found that satisfactory miniature hose may be made from the readily crimpable filaments of this invention without the added steaming operation which has been required in the past for bicomponent filament stretch hose.

The expression "relative viscosity" as used herein signifies the ratio of flow time in a viscometer of a polymer solution containing 8.2 percent by weight of polymer, relative to the flow time of the solvent by itself. Measurements of relative viscosity are made with 5.5 grams of polyamide in 50 milliliters of 90 percent by weight formic acid at 25°C.

Shrinkage and crimp elongation of the filament are determined as follows:

A 750 denier skein of monofil or multifilament yarn is prepared by winding the requisite number of turns on a reel to give a skein of about 55 centimeters length when suspended with a weight attached. The denier of the filament bundle representing the collapsed skein will, of course, be twice that of the original skein, i.e., 1,500 denier. The skein is hung on a hook with a 500 gm. weight suspended from its other end. After one minute, the length (a) of the skein is measured. The 500 gm. load is removed and a 1.8 gm. load is applied in its place so that the skein is under a tensile load of 1.2 mg./den. (mgd), i.e., a tension slightly in excess of that on the yarn when knitted into a fabric. The skein with the weight attached is subjected to 100°C. steam at atmospheric pressure (hereinafter referred to as "atmospheric steam") for one minute, after which the skein is allowed to dry in air for 10 minutes. The skein length (b) is then measured. The 1.8 gm. load is then removed, the 500 gm. load is again applied for one minute, and the length (c) of the skein determined. The crimp elongation and shrinkage of the filament are calculated from the following equations:

$$\text{Crimp Elongation, \%} = 100 \frac{c - b}{b}$$

$$\text{Shrinkage, \%} = 100 \times \frac{a - c}{a}$$

The crimp diameter of the filament under a tension of 1.2 mgd is determined by taping 1 inch lengths of the crimped tensioned skein on a microscope slide and projecting the magnified image on a grid covered screen by means of a projection microscope.

The differential thermal analysis (DTA) melting point of the polymer is determined with a commercially available Du Pont 900 Thermal Analyzer using a Scanning Calorimeter head. Some instruments are designed to measure both endothermic (melting) and exothermic (freezing) temperatures; however, only the endothermic temperatures are used for values reported herein. Most polymers, and particularly copolymers, melt over a temperature range depending on the heating rate. In this determination, the melting point is taken as the peak temperature in the endothermic temperature plot. Due to the fact that polymer melting temperatures are usually not sharp, the accuracy of this measurement is  $\pm 2^\circ \text{C}$ . The polymer sample may be in the form of flakes, chips, fiber or film. In the following examples, the polymer samples were in the form of flakes or fiber. Using the instructions provided with the commercial Du Pont instrument, the conditions used to make the measurements are as follows:

Reference - Aluminum Pan

Program Mode - Heating

Heating Rate - 12°C./min.

Atmosphere - Nitrogen, 6 min.

T Scale - 50°C./in.

T Shift - 0

Δ T Scale - 0.1°C./in.

Δ T Shift - 0

Amide group frequency is calculated as follows:

1. Homopolyamides

a. AABB polymers (e.g., 6-6 or 6-12 nylons)

$$F = \frac{2 \times 10^6}{W_m}$$

5 where

F = Amide Frequency

W<sub>m</sub> = Gram molar weight of polyamide repeat unit.

Thus,

$$F_{6-6} = \frac{2 \times 10^6}{226} = 8850$$

$$F_{6-12} = \frac{2 \times 10^6}{310} = 6450$$

15 b. AB polymers (i.e., 6 nylon)

$$F = \frac{10^6}{W_m}$$

20 Thus,  $F_6 = \frac{10^6}{113} = 8850$  (same as for 6-6)

2. Copolyamides

$$F = f_1 F_1 + f_2 F_2 + \dots$$

25 Where

f<sub>i</sub> is the weight fraction of polyamide 1 and F<sub>i</sub> is its amide frequency, etc.

(Note: All copolyamides of 6-6/6 have an amide frequency of 8850)

30 Thus, for 6-6/6-12 (75:15:10)

$$F = (f_{6-6} + f_{6-12}) 8850 + f_{6-12} \times 6450 \\ = 0.90 \times 8850 + 0.10 \times 6450 \\ = 8610$$

#### EXAMPLE I

35 An evaporator is charged with an aqueous solution containing 257 pounds (116.6 kg.) of hexamethylenediammonium dodecanedioate (6-12 nylon salt), 2034 pounds (922.6 kg.) of hexamethylenediammonium adipate (6-6 nylon salt) and

40 338 pounds (153.3 kg.) of epsilon caprolactam, and the resulting solution is heated at 34.7 psig (3.4 atmospheres) until the temperature reaches 146°C., giving a salt concentration of approximately 76 percent. The solution is then transferred to an autoclave, heated to a temperature of about 205°C. and brought to a pressure of 250 psig (18 atmospheres). At this point, sufficient 20 percent aqueous titanium dioxide slurry is added to give a delusterant concentration of 0.3 percent TiO<sub>2</sub> in the final copolymer. The solution is then heated at 250

45 psig until the temperature reaches 230°C. The pressure is then reduced over a period of 80 minutes to atmospheric, and the temperature is increased to 250°C. The copolymer is then held, at atmospheric pressure, for 30 minutes at a temperature of 250° - 260°C., extruded under 90 psig (7.1 atmospheres) nitrogen in the form of continuous strands, quenched with water and cut into flake. The copolymer, consisting by weight of 75 percent polyhexamethylene adipamide, 15 percent polyepsilon caproamide and 10 percent polyhexamethylene dodecanedioamide, has a relative viscosity of 46.

50 60 Polyhexamethylene adipamide (6-6 nylon) flake having a relative viscosity of 46.5 is prepared in the conventional manner. The two flakes (6-6 and 6-6/6-12) are first conditioned by exposure to humidified nitrogen at 125°C. and 145°C., respectively, and then melted and pumped to a spinneret assembly of the type shown in FIG. 3 of U.S. Pat. No. 3,399,108 to Olson, with holes arranged to spin three filament

65 yarns. The relative viscosity of the 6-6 polymer after conditioning is 50 and that of the 6-6/6-12 copolymer flake is 56. The two polymers are extruded, with the copolymer as the

70 core to form eccentric sheath-core three-filament hosiery yarns containing 58 percent of the random copolymer and 42 percent by weight of the homopolymer. The sheath, at its thinnest point, has a thickness equivalent to about 1 percent of the total filament diameter. The clearance between the projection 75 135 and plate 142 of Olson is 0.003 inch (0.076 mm.). The

filaments are set by quenching, using a 60 inch (152 cm.) chimney and an air temperature of 60° C., steam conditioned as described by Babcock in U.S. Pat. No. 2,289,860 and wound into a package at 546 ypm. The yarn is subsequently withdrawn from the package and drawn at a ratio of 4.47 over an unheated draw pin situated between feed and draw rolls to give a final denier of 23-24 (nominally 20-3). It is then passed from the draw roll at 584 ypm (533 meters/min.) through a 3-inch long (7.6 cm.) tubular crimping chamber of the type shown in FIG. 5 of the Olson patent. The yarn is heated by passing 1.05 cubic feet/minute (0.03 cu. meter/min.) of 278° C. air through the chamber to give an air temperature of 188° C. at the exit.

The yarn is then passed over two snubbing pins, the total yarn contact with the pins being 390°, then to a withdrawal roll and finally to a winding device. The snubbing pins act to reduce the speed of the yarn in the heating zone so that the components can shrink differentially and the filaments can crimp under the influence of the heat. In addition, the yarn is stretched sufficiently between the pins and the withdrawal roll to remove most of the crimp. Between the draw and withdrawal rolls, the yarn is permitted to retract by 40 percent of its as-drawn length.

When the crimpable yarn is exposed to hot water or steam, it crimps again in a very uniform fashion, and the crimp diameter and crimp elongation are quite uniform. The crimp elongation at a load of 1.2 mgd, determined as described previously, is 38 percent in atmospheric steam. The average crimp spacing and diameter are about 22 mils (0.56 mm.) and 4.6 mils (0.12 mm.), respectively. The shrinkage of the yarn is 1.6 percent. The tenacity of yarn removed from finished hose is 4.2 gpd.

#### EXAMPLE II

20 denier, three-filament yarn with a crimp elongation of 40 percent, prepared substantially as described in Example I, was used as the leg yarn in conventional knitting of women's hose. For comparison, otherwise identical hose were knit from 20 denier, three filament yarn prepared from the composition described below in the last paragraph of Example III. It was observed that greige hose from the yarn of this invention were substantially smaller than the comparison hose after removal from the knitting machine due to a tendency for the filaments to crimp at this stage. This reduction in size leads to a reduction in picks during subsequent handling of the hose in the mill. When the above two types of hose are tested for picking propensity by tumbling greige hose for six minutes in a drum lined with pins designed to produce picks at a rapid rate, the number of picks produced in 12 hose of the yarn of this invention is 101 compared to 226 for 12 of the comparison hose. In addition, it was found, however, that the tumble steaming operation could be eliminated for the hose from the readily crimpable yarn of this invention since the crimp development during the normal scouring and dyeing operation was sufficient. When hose from the yarn of this invention, without tumble steaming, is scoured at 150° F. (65.6° C.) or 212° F. (100° C.) for 15 minutes, followed by a standard dye cycle at 180° F. (82.2° C.) for 90 minutes, the average over-all length of the unboarded hose was approximately 19 inches (48 cm.), and the length of the leg portion was approximately 15 inches (38 cm.). The average over-all length of the comparison hose with tumble steaming was about 21 inches (60 cm.), and the leg length was 17 (50 cm.) inches.

#### EXAMPLE III

A copolymer flake containing 75 percent by weight of hexamethylene adipamide polymer units, 15 percent epsilon caproamide units and 10 percent hexamethylene dodecanedioamide units and having a relative viscosity of 55.9 is prepared following the general procedure of Example I.

The copolymer flake and 6-6 nylon polymer flake having a relative viscosity of 50.1 are extruded from a spinneret of the type identified in Example I to form a sheath-core filament

with the copolymer as the core and having a final denier of about 15. The monofil, consisting of about 60 percent core and 40 percent sheath by weight, is air-quenched and wound into a package. The filament is then removed from the package and drawn at a ratio of 5.02 over an unheated pin at a draw roll peripheral speed of 850 yds./min. (776 meters/minute). From the draw roll, the filament is passed upwardly through a tubular crimping chamber of the type shown in FIG. 5 of the Olson patent, over a change-of-direction guide, downwardly to a series of snubbing pins of 3/16 in. (4.77 mm.) diameter and over a power-driven withdrawal roll rotating at a peripheral speed of 527 yds./min. (482 meters/min.) to a winding device where the filament is wound into a package in the usual manner. In the crimping device, the filament is heated by a stream of air which is passed into the jet at a temperature of 295° C.

Filaments designated A and B in Table I are prepared with different amounts of snubbing. Withdrawal roll speed is somewhat higher for filament B, as indicated by the lower extent of retraction. The cumulative snubbing angle, i.e., the sum of the angles of contact with the individual pins, is reported in Table I. Crimp characteristics and tensile properties of the filaments are also reported in Table I.

For comparison, filaments are prepared substantially as was filament B except that the core is a copolymer prepared substantially as in Example VIII of Olson by combining a 49.5 percent by weight 6-6 salt solution containing 1,362 lbs. of dry salt, a 26 percent by weight 6-12 salt solution containing 486 lbs. of dry salt and a 31 percent by weight 6-10 salt solution prepared with technical grade sebacic acid and containing 833 lbs. of dry salt. The draw ratio is adjusted to give approximately the same elongation at break as the filaments of this invention. The air temperature at the crimping chamber is also slightly lower since this temperature was more nearly optimum for polymer composition. These filaments are designated C and D in the following table.

TABLE I

| Filament                                               | A     | B     | C     | D     |
|--------------------------------------------------------|-------|-------|-------|-------|
| Draw Ratio                                             | 5.02  | 5.02  | 4.74  | 4.74  |
| Snubbing, Cumulative Angle                             | 245°  | 1025° | 245°  | 1025° |
| Retraction*, %                                         | 38    | 28    | 28    | 28    |
| Crimping Jet Inlet Air Temp., °C.                      | 295   | 295   | 280   | 280   |
| Crimp Elongation, %                                    | 58    | 71    | 41    | 63    |
| Crimps/inch, Extended, 0.3 g.p.d. load                 | 29.0  | 37.8  | 28.5  | 41.6  |
| Crimps/cm., Extended, 0.3 g.p.d. load                  | 11.4  | 14.9  | 11.2  | 16.4  |
| Shrinkage, %                                           | 3.0   | 3.7   | 5.3   | 4.6   |
| Crimp Pitch, Mils                                      | 22.2  | 15.1  | 25.5  | 14.6  |
| Crimp Pitch, mm.                                       | 0.565 | 0.384 | 0.648 | 0.371 |
| Crimp Dia., Mils                                       | 7.1   | 4.3   | 7.9   | 4.4   |
| Crimp Dia., mm.                                        | 0.180 | 0.109 | 0.200 | 0.112 |
| Tenacity, gpd.                                         | 5.3   | 5.1   | 4.4   | 3.8   |
| Elongation**, %                                        | 43    | 45    | 45    | 50    |
| Tenacity, gpd, After Boil-off                          | 4.5   | 5.1   | 3.9   | 3.3   |
| Elongation**, %                                        | 42    | 44    | 45    | 38    |
| DTA Melting Point, °C., copolyamide                    | 219   | 219   | 207   | 207   |
| Amide Freq., Equiv./10 <sup>6</sup> grams, copolyamide | 8595  | 8595  | 7840  | 7840  |

\*Retraction of filament between draw roll and withdrawal roll based on peripheral speeds of rolls.

\*\*Elongation at break

Women's seamless hose are knit in the conventional manner using 15 denier monofil prepared substantially as described in connection with filaments C, D and B in Example III. It was noted that the greige hose as removed from the knitting machine were much smaller in the case of filaments D and B as compared to hose from filament C. Table 2 records the relative areas of the knit hose tubing where the area of the hose from filament C is designated as 1.00. This reduction in fabric area is due to the greater tendency of filaments D and B to crimp after knitting. Although the relative area of the fabric from filament D is substantially reduced, this is accomplished only with a considerable (0.6 gpd) reduction in tenacity, as can be seen from a comparison of filaments C and D of Table 1.

TABLE 2

| Filament | Relative Area | Area Reduction, % |
|----------|---------------|-------------------|
| C        | 1.00          | —                 |
| D        | 0.35          | 65                |
| B        | 0.31          | 69                |

## EXAMPLE V

Following the procedure of Example III, copolyamides of 6-6, 6 and 6-12 nylon having the compositions shown in Table 3 were prepared and processed into 15 denier bicomponent monofilaments with 6-6 nylon as the sheath component, the processing conditions being substantially as in Example I. Table 3 records the crimp elongation values for the three compositions, the 75:15:10 and 70:20:10 compositions

being within the scope of this invention while the 82:8:10 composition is for comparison.

TABLE 3

|    | 6-6/6-12 Composition, weight %                     | 75:15:10 | 70:20:10 | 82:8:10 |
|----|----------------------------------------------------|----------|----------|---------|
| 5  | DTA Melting Point, °C.                             | 219      | 215*     | 234*    |
| 10 | Amide Group Freq.,<br>Equiv./10 <sup>6</sup> grams | 8610     | 8610     | 8610    |
|    | Crimp Elongation, %                                | 66       | 63       | 30      |

\*Determined from phase diagram

15 Having thus described the invention, what is claimed as new and desired to be secured by Letters Patent is:

1. A readily crimpable yarn of at least one composite filament having continuous, adherent, eccentric components, one component being a polyamide, the other a random copolyamide containing 70-82 percent by weight of hexamethylene adipamide units, 13-25 percent by weight of caproamide units and 5-17 percent by weight of hexamethylene dodecanedioamide units.
- 25 2. The yarn of claim 1, said filament being characterized by a shrinkage in the fabric of less than 4 percent.
3. The yarn of claim 2, said filament having an after boil-off tenacity of at least 4.0 grams/denier.
4. The yarn of claim 2, said copolyamide having a DTA 30 melting point of 210°-225° C.
5. The yarn of claim 2, said one component being polyhexamethylene adipamide, said copolyamide containing the three different units in a ratio of about 75:15:10.

\* \* \* \* \*

35

40

45

50

55

60

65

70

75